

## UNITED STATES PATENT OFFICE

2,458,397

DYEING OF NYLON FIBERS BY TREATING  
WITH NITROGENOUS CONDENSATION  
PRODUCTSJames Hutchison MacGregor, Bocking, Braintree,  
England, assignor to Courtaulds Limited, Lon-  
don, England, a British companyNo Drawing. Application October 12, 1944, Se-  
rial No. 558,469. In Great Britain November  
18, 1943

5 Claims. (Cl. 8—31)

1

This invention relates to the dyeing of nylon fibres with direct cotton dyestuffs in an acid dye-bath.

In British Specification No. 547,844, Courtaulds Limited, C. M. Whittaker and C. C. Wilcock have described a process for dyeing nylon with direct cotton dyestuffs in an acid dyebath by carrying out the dyeing in the presence of an organic compound which increases the affinity of the nylon for the dyestuffs. The list of organic compounds in the specification includes cyanamide, guanidine, arylguanidines, dicyandiamide, di-cyandiamidine and melamine.

I have now found that nylon fibres containing a water-insoluble condensation product of formaldehyde and cyanamide or a derivative thereof can be dyed with a direct cotton dyestuff from an acid dyebath with a considerably enhanced rate of absorption. The water-insoluble condensation product may be incorporated in the nylon fibres by treating the said fibres with an aqueous solution containing formaldehyde and cyanamide or a derivative thereof, either as such or in the form of a water-soluble precondensate, and subsequently heating to convert the water-soluble condensation product into the insoluble form.

Cyanamide derivatives which may be used in the present invention are dicyandiamide, melamine, guanidine, biguanide and dicyandiamidine or alkyl, hydroxyalkyl or aryl substitution products of guanidine, biguanide and dicyandiamidine. Salts of any of these compounds may be used in preparing the impregnating solution.

When carrying out the present invention, I prefer to employ a padding process and in this case to use a padding liquor containing in each litre not more than about 20 grams of the cyanamide formaldehyde compound. If a more concentrated solution is used in the padding process, there is a tendency during the subsequent dyeing process for precipitation of a complex compound of the dyestuff and the cyanamide-formaldehyde condensate to take place, with the consequent production of weak and uneven dyeings.

The process of the present invention is of particular value when it is desired to use direct cotton dyestuffs, such as Chlorazol Fast Pink BKS (Colour Index No. 353) and Chlorazol Black BHS (Colour Index No. 401), which are absorbed very slowly by untreated nylon fibres. The wash fastness of the dyeings obtained by the process of the present invention is extremely good and this result is obtained without impairment of

2

the light fastness. The nylon fibres, particularly in the form of fabric, treated according to the present invention lose more or less of their characteristic "soapy" handle.

5 The following examples illustrate the nature of the present invention without the invention being limited to these examples.

*Example 1*

10 A length of an all nylon fabric is padded through an aqueous solution containing 10 grams of diphenylguanidine (dissolved in 10 cubic centimetres of 80 per cent acetic acid) and 50 cubic centimetres of 40 per cent formaldehyde in each 15 litre of solution, at ordinary room temperature, squeezed evenly, so that the fabric retains approximately 70 per cent of its own weight of padding solution, dried at under 100° centigrade and finally heated at 140° centigrade for 10 minutes. 1 kilogram of the so-treated nylon fabric is then entered at a temperature of 90° centigrade into 50 litres of a dyebath containing 2 per cent of Chlorazol Fast Pink BKS and 7.5 per 20 cent of 80 per cent acetic acid calculated on the weight of nylon, and dyeing continued at this 25 temperature for one hour. A full shade of pink, which is very fast to washing, is obtained, while the dyebath is almost exhausted. A piece of untreated fabric gives a much paler shade of pink 30 when dyed under similar conditions. Furthermore, the treated fabric possesses a less soapy handle than the untreated fabric.

*Example 2*

35 A length of an all nylon fabric is padded through an aqueous solution containing 15 grams of dicyandiamide and 150 cubic centimetres of 40 per cent formaldehyde in each litre of solution at ordinary temperature, squeezed evenly so that the fabric retains approximately 70 per cent 40 of its own weight of padding solution, dried at under 100° centigrade and finally heated at 140° centigrade for 10 minutes. 1 kilogram of the so-treated fabric is then entered at a temperature of 90° centigrade into 50 litres of a dyebath containing 2 per cent of Chlorazol Fast Pink BKS and 7.5 per cent of 80 per cent acetic acid, calculated on the weight of nylon, and dyeing continued at this temperature for one hour. A full shade of pink which is very fast to washing 45 is obtained, while the dyebath is practically exhausted.

*Example 3*

A length of an all nylon fabric is padded 55 through an aqueous solution, containing 10 grams

of guanidine adipate and 150 cubic centimetres of 40 per cent formaldehyde in each litre of solution, at ordinary temperature, squeezed evenly so that it retains approximately 70 per cent of its own weight of padding solution, dried at under 100° centigrade and finally heated at 140° centigrade for 10 minutes. 1 kilogram of the so-treated fabric is then entered at a temperature of 90° centigrade into 50 litres of a dyebath containing 1 per cent of Chlorazol Black BHS and 7.5 per cent of 80 per cent acetic acid, calculated on the weight of nylon and dyeing continued at this temperature for one hour. A full shade is obtained and the dyebath is well exhausted. The fastness to washing of the dyeing is extremely good. Untreated nylon dyed under similar conditions to those just described is dyed a very pale shade.

*Example 4*

43 denier/17 filament scoured bright nylon yarn is padded through an aqueous solution containing 20 grams of monoethanol biguanide neutral sulphate and 150 cubic centimetres of 40 per cent formaldehyde in each litre of solution, at ordinary room temperature, squeezed evenly so that yard retains approximately 70 per cent of its own weight of padding solution, dried at under 100° centigrade and finally heated at 140° centigrade for 10 minutes. 1 kilogram of the so-treated yarn is then entered at a temperature of 90° centigrade into 50 litres of a dyebath containing 1 percent of Chlorazol Fast Pink BKS and 7.5 per cent of 80 per cent acetic acid, calculated on the weight of nylon, and dyeing continued at this temperature for one hour. A full shade of pink is obtained and the dyebath is well exhausted. The fastness to washing of the dyeing is extremely good.

What I claim is:

1. A process for dyeing nylon fibres at an enhanced rate of absorption with direct cotton dyestuffs having little affinity for nylon which comprises incorporating in the nylon fibres a water-insoluble condensation product of formaldehyde and a member of the group consisting of cyanamide, dicyandiamide, melamine, guanidine, biguanide, dicyandiamidine, alkyl, hydroxy-alkyl, and aryl substituents of guanidine, biguanide and dicyandiamidine and dyeing the fibres with the direct cotton dyestuff from an acid dyebath.

2. A process for dyeing nylon fibres at an enhanced rate of absorption with direct cotton dyestuffs having little affinity for nylon which comprises treating the nylon fibres with an aqueous solution containing formaldehyde and a member of the group consisting of cyanamide, dicyan-

diamide, melamine, guanidine, biguanide, dicyandiamidine, alkyl, hydroxyalkyl and aryl substituents of guanidine, biguanide, and dicyandiamidine, converting the formaldehyde and member of the group into a water-insoluble condensation product and dyeing the fibres with the direct cotton dyestuff from an acid dyebath.

3. A process for dyeing nylon fibres at an enhanced rate of absorption with direct cotton dyestuffs having little affinity for nylon which comprises treating the nylon fibres with an aqueous solution containing formaldehyde and cyanamide, converting the formaldehyde and cyanamide into a water-insoluble condensation product and dyeing the fibres with the direct cotton dyestuff from an acid dyebath.

4. A process for dyeing nylon fibres at an enhanced rate of absorption with direct cotton dyestuffs having little affinity for nylon which comprises treating the nylon fibres with an aqueous solution containing formaldehyde and diphenylguanidine, converting the formaldehyde and diphenylguanidine into a water-insoluble condensation product and dyeing the fibres with the direct cotton dyestuff from an acid dyebath.

5. A process for dyeing nylon fibres at an enhanced rate of absorption with direct cotton dyestuffs having little affinity for nylon which comprises treating the nylon fibres with an aqueous solution containing formaldehyde and guanidine adipate, converting the formaldehyde and guanidine adipate into a water-insoluble condensation product and dyeing the fibres with the direct cotton dyestuff from an acid dyebath.

JAMES HUTCHISON MACGREGOR.

REFERENCES CITED

The following references are of record in the file of this patent:

UNITED STATES PATENTS

| Number    | Name      | Date          |
|-----------|-----------|---------------|
| 2,119,189 | Widmer    | May 31, 1938  |
| 2,168,336 | Heckert   | Aug. 8, 1939  |
| 2,234,905 | Tallis    | Mar. 11, 1941 |
| 2,253,457 | Whittaker | Aug. 19, 1941 |
| 2,317,965 | Bestian   | Apr. 27, 1943 |
| 2,347,143 | Wilcock   | Apr. 18, 1944 |
| 2,356,677 | MacGregor | Aug. 22, 1944 |

FOREIGN PATENTS

| Number  | Country       | Date           |
|---------|---------------|----------------|
| 547,844 | Great Britain | Sept. 14, 1942 |

OTHER REFERENCES

55 Stott, "Dyeing of Nylon Fibres," article in American Dyestuff Reporter for Oct. 2, 1939, pages P582-P584.

**Certificate of Correction**

Patent No. 2,458,397.

January 4, 1949.

JAMES HUTCHISON MacGREGOR

It is hereby certified that errors appear in the printed specification of the above numbered patent requiring correction as follows:

Column 3, line 3, before the word "temperature" insert *room*; line 26, strike out "yard" and insert instead *the yarn*; and that the said Letters Patent should be read with these corrections therein that the same may conform to the record of the case in the Patent Office.

Signed and sealed this 31st day of May, A. D. 1949.

[~~SEAL~~]

THOMAS F. MURPHY,  
*Assistant Commissioner of Patents.*